

## UNITED STATES PATENT OFFICE.

JOHN K. SHAW, OF MINNEAPOLIS, MINNESOTA.

## PROCESS OF OBTAINING FIBERS FROM BAGASSE.

No Drawing. Application filed October 23, 1920, Serial No. 419,046. Renewed January 20, 1923.

*To all whom it may concern:*

Be it known that I, JOHN K. SHAW, a citizen of the United States, residing at Minneapolis, in the county of Hennepin and State of Minnesota, have invented certain new and useful Improvements in Processes of Obtaining Fibers from Bagasse; and I do hereby declare the following to be a full, clear, and exact description of the invention, such as will enable others skilled in the art to which it appertains to make and use the same.

This invention relates to a process for treating bagasse and analogous fibers and has for its object to provide a method which will produce both wall board making fibers as well as paper making fibers from bagasse and analogous raw material at a minimum of cost.

With these and other objects in view the invention consists in the novel steps and combinations of steps constituting the process all as will be more fully hereinafter disclosed and particularly pointed out in the claims.

In order that the precise invention may be the more clearly understood it is said:— In my copending application Sr. No. 419,044 filed, Oct. 23, 1920, and entitled Process of making bagasse and analogous fibers, I have disclosed a procedure wherein bagasse fibers are only partially cooked so that they make a superior fiber for wall board purposes but are not suitable for paper making purposes.

According to the process of this said copending application the bagasse fibers are only cooked to such a degree as will be sufficient to loosen up their encrusting casing, but insufficient to dissolve out their natural pith. By this procedure, the bagasse fibers are obtained in an unusually resilient and strong condition, for making wall boards, while their natural pith which is not destroyed is found to be a very efficient heat insulator and to add very materially to the yield of board making substance. By the term "encrusting casings" found in the description and claims is meant what appears to be a more or less stiff and brittle fibrous casing to which the relatively flexible and strong fibers are found to be attached when dry bagasse is observed under a magnifying glass. I believe the fibers of this casing are made up of those forming the outer skin, or wall, of the stalk, and

are substantially free from pith cells, while the said more flexible fibers are found farther inside the stalk and are associated with numerous pith cells. Whatever may be the true nature of this so called casing, it is a fact that it constitutes a brittle mass which, when mechanically removed, frees the more flexible fibers and renders them suitable for the purpose in hand.

The prior processes on the other hand, have invariably destroyed this valuable pith material, either mechanically or chemically, and they have also injured to a greater or less extent the strength of the ultimate fibers, all as is set forth in said copending application.

In carrying out this invention, on the other hand, I first proceed to only partially cook the bagasse and analogous fibers in the same manner as is disclosed in said copending application. That is, I subject said fibers to any suitable chemical such as an alkali, a sulphate, or a sulphite, and cook the same only so long as is necessary to loosen up the encrusting casing of said fibers and I am careful not to prolong the cooking sufficiently to dissolve out a substantial portion of the valuable natural pith with which said fibers are accompanied. I thus not only use up a minimum quantity of chemicals but I preserve the valuable wall board making pith.

After the bagasse and analogous fibers have been thus only partially cooked, I subject the same to the action of a suitable beating engine, whereupon I recover a portion of the longer partially cooked fibers with their natural pith and mechanically separate this said portion from the shorter fibers also accompanied by their natural pith.

The shorter fibers which are not separated from the natural pith are used for board making purposes precisely as is disclosed in my said copending application above mentioned, but may also have added thereto the dissolved cellulose constituents and pith of said longer fibers as will presently appear. The first mentioned portion of fibers, however, which also has not as yet been separated from its natural pith, I further cook in any suitable chemical solution to such an extent as will dissolve said pith and form paper making fibers therefrom.

These said fully cooked fibers are found to make a very high grade pulp from which

a superior grade of paper can be manufactured. It will now be clear that by following the procedure above outlined, I avoid dissolving a large portion of the pith in treating bagasse fibers, and therefore avoid the great loss of cellulosic material that has been heretofore experienced by practicing other cooking processes and by saving this pith with the board making fibers, all loss of the same is avoided because the mechanical separation of the two classes of fibers saves not only the pith but a considerable amount of the short fibers which are valuable for the manufacture of said heat insulating wall boards.

While it is true that some of the cellulose material of the long fibers will be lost during the second cooking, yet, this loss does not amount to anything like the total loss that is experienced in the prior processes, whether the pith is mechanically stripped from the fibers before the cooking, or is completely dissolved therefrom during the cooking.

It is found in practice that it takes a less weight of chemicals to make a ton of paper making pulp by this process than by the prior processes, and the said valuable board making material is obtained in addition as a by product.

It is obvious that those skilled in the art may vary the details of the procedure without departing from the spirit of the same, and therefore, it is not desired to be limited to

the above disclosure except as may be required by the claims.

What is claimed is:

1. The process of treating bagasse and analogous fibers which consists in cooking said fibers with their natural pith sufficiently to loosen their encrusting casings but insufficiently to dissolve a substantial portion of said pith; subjecting said fibers to the action of a beating engine; separating out a portion of the long fibers from the short fibers present after leaving said engine; and subjecting said portion of long fibers to a second cooking action to produce a paper making pulp, substantially as described.

2. The process of treating bagasse and analogous fibers which consists in cooking said fibers with their natural pith sufficiently to loosen their encrusting casings but insufficiently to dissolve a substantial portion of said pith; subjecting said fibers to the action of a beating engine; separating out a portion of the long fibers from the short fibers present after leaving said engine; subjecting said portion of long fibers to a second cooking action to produce a paper making pulp; and a solution of the pith accompanying said long fibers; recovering said short fibers; forming the same into a board; and applying thereto said solution, substantially as described.

In testimony whereof I affix my signature.

JOHN K. SHAW.